

Aug. 9, 1966

F. J. KOVARIK

3,264,705

P. J. KOVARI  
PROCESS FOR IMPROVING THE PILL RESISTANCE OF  
TWO-COMPONENT ACRYLONITRILE POLYMERS

Filed Sept. 8, 1960

2 Sheets-Sheet 1

FIG. 1



FIG. 2



INVENTOR  
FRANK JOSEPH KOVARIK

BY

BY *Sol Schwartz* ATTORNEY

**ATTORNEY**

Aug. 9, 1966

F. J. KOVARIK

3,264,705

PROCESS FOR IMPROVING THE PILL RESISTANCE OF  
TWO-COMPONENT ACRYLONITRILE POLYMERS

Filed Sept. 8, 1960

2 Sheets-Sheet 2

FIG. 3



FIG. 1A



FIG. 7



FIG. 6



FIG. 5



INVENTOR  
FRANK JOSEPH KOVARIK

BY *Sol Schwartz*  
ATTORNEY

3,264,705

**PROCESS FOR IMPROVING THE PILL RESISTANCE  
OF TWO-COMPONENT ACRYLONITRILE POLY-  
MERS**Frank Joseph Kovarik, Waynesboro, Va., assignor to E. I.  
du Pont de Nemours and Company, Wilmington, Del.,  
a corporation of DelawareFiled Sept. 8, 1960, Ser. No. 54,697  
5 Claims. (Cl. 28—76)

This invention relates to improved crimped composite filaments and a process of making them.

It has been proposed to produce helically crimped composite synthetic polymeric filaments having the capacity of changing the amount of crimp upon being exposed to the effect of a swelling agent and upon reverting to the original crimp upon removal of the swelling agent. This characteristic is, for convenience, referred to as "reversible" crimp and is observed by the "squirming" of the filaments upon both application and removing of the swelling agent. The value of this crimp reversibility is evidenced by the ability of the filaments in yarns, when embodied in a fabric, to squirm or twist around in the fabric under the influence of a swelling agent such as water (and also on removal of the swelling agent), but, nevertheless, to regain the original crimp in the fabric with removal of the swelling agent, as by drying. Fabrics containing these filaments acquire a high degree of fullness or covering power as a result of the swelling treatment and retain or even increase this fullness after being subjected to such treatments repeatedly.

It has been found that the high degree of crimp reversibility in the fibers necessary to produce yarns and fabrics with good bulk, compressional resilience, response to finishing treatments, and recovery from glazing is generally accompanied by a high level of crimp frequency. This high level of crimp frequency leads to a rough wool-like handle in knit-wear and woven-wear fabrics and does not afford soft fabrics similar to those made from cashmere, for example.

For some applications, especially in fabrics from woolen-spun yarns, the use of these recent fibers is restricted by a phenomenon known as "pilling."

One object of this invention is to produce a crimped composite filaments that affords fabrics that are density stable to washing and ironing and are pill resistant.

Another object is to produce composite filaments having a reversible crimp and a low level of crimp that affords soft, cashmere-like fabrics.

These and other subjects are accomplished as described more fully below.

Filaments of the invention consist of at least two fiber-forming compositions of polymers of acrylonitrile in eccentric relationship at least one of which contains 50 or more milliequivalents per kilogram of polymer of ionizable groups in excess of the ionizable groups contained in the other components. After the filaments are extruded and the fiber structure established, the solidified fibers are drawn from 1.1 to 10 $\times$  and relaxed in the presence of a plasticizing medium such as steam under a tension of at least 0.01 gram per denier. The extent of relaxation should be at least 50% of the boil-off shrinkage of the as-drawn yarn prior to drying the filaments. After relaxation, the fibers are mechanically crimped if desired, then dried and given a hot relaxation treatment to permit the development of a helical crimp.

More specifically, the composite filament comprises at least 2 polymers of acrylonitrile eccentrically disposed toward each other and has 5 to 10 helical crimps per inch of extended length, a crimp product of less than 100, a crimp reversibility (ECR) of 25-50%, a tenacity of at least 2 grams per denier and is characterized by a high

resistance to pilling when spun into yarn and knitted or woven into a fabric.

The amount of relaxation may vary from 50 to 99+% of the boil-off shrinkage of the as-drawn yarn. Preferably a relaxation of at least 75% of the boil-off shrinkage of the as-drawn yarn is used. "Boil-off" shrinkage is that fiber shrinkage which takes place upon exposure to boiling water for a period of at least about 5 minutes.

The length of time of the relaxation treatment is not critical and may be from 0.5 second to 10 minutes. Preferably, this is from 0.5 to 2 seconds when it is used as part of a continuous process.

The relaxation can take place in any type of heating medium having a temperature of about 100° C. which has a plasticizing action on the yarn such as organic vapors, or steam. Steam at pressures of from 0 to 5 p.s.i. gage is preferably used. Temperatures as high as 120° C. may be used.

The process can be continuous or batch. Preferably the relaxation is done continuously in conjunction with a wash-drawing process as this affords lower crimp levels. The beneficial results of pill reduction of fabrics containing the fibers may also be obtained by a batch process wherein the drawn and wet filaments are lagged in some manner as in cans before the relaxation step.

The process is most advantageously used on tows of 5,000 to 450,000 denier.

By the expression "polymer of acrylonitrile" is meant the homopolymer of acrylonitrile or copolymers of acrylonitrile and monoethylenically unsaturated addition type monomers containing at least 80% acrylonitrile. Suitable comonomers include the ethylenically unsaturated sulfonic acids as methallyl sulfonic acids and others as disclosed in U.S. Patents 2,527,300 and 2,601,256 and other monomers as disclosed in Jacobson U.S. 2,436,926 and in Arnold U.S. 2,456,360.

The two polymers selected as components must have the required difference in shrinkage and in swellability so that the composite filament crimps and a reversible crimp results. To develop crimp in the composite filaments, the shrinkability of one component should be at least 0.2% greater than the shrinkability of the other component, that is, said component has at least 0.2% greater loss of the original length upon shrinkage than

the other component. The shrinkability of a component is determined by measuring the shrinkage, upon immersion in boiling water under no tension, of a monocomponent filament made from the component polymer (spun and otherwise processed under substantially the same conditions as the composite filament). One component of the crimped filament should have a reversible length change after shrinkage of at least 0.05% and preferably at least 0.10% more than that of the other component, that is, said component has at least 0.05% greater change in length

of the original length upon swelling than the other component. The reversible length change of a component is determined by measuring the increase in length of a monocomponent filament of the component polymer (spun and subjected to after-treatments under the same conditions as the composite filament) upon being immersed in the aqueous medium used for the testing of the crimp reversibility of the composite filament. Measurements are obtained with strands of approximately 100 denier and approximately 15 inches long as follows: The samples (previously relaxed by a boil-off) are clamped in a tensile tester with a small amount of slack and held in the proper medium (air, cold water, or hot water) for about 2 minutes. The mechanically driven clamp is then started at a low rate of elongation (0.3 inch per minute);

it is stopped and reversed immediately when the stress-strain curve starts to depart from the zero line. The true length of the sample is then calculated from the clamp

distance in the starting position and the chart distance between the start of the test and the point where the stress-strain curve began.

After wet tests the samples are dried (while clamped) by means of a hair dryer, and the length of dry strand at room temperature determined as above. Wet to dry cycles are repeated until the length change becomes constant. As a rule some shrinkage occurs during the first cycle. For most samples, satisfactory results are obtained with three cycles.

The reversible length change is calculated in percent, based on the final dry length of the sample.

$$\text{Reversible length change} = \frac{\text{length wet} - \text{length dry}}{\text{final length dry}} \times 100$$

Results from at least four different strands are averaged to obtain a representative value. Suitable polymers, methods for selecting them, and crimping methods such as by heat, boil-off or steam are described in coassigned and copending Taylor application, Serial No. 771,677, filed November 3, 1958, now U.S. Patent 3,038,237.

The crimp reversibility of the composite filaments of this invention is determined by the following test.

A single filament is separated from the single end or tow of drawn, unrelaxed fibers. A three-inch length of the filament is attached to opposite sides of a rectangular copper wire frame with 30% slack between the ends. The rack and filament is then boiled off for 15 minutes to develop the crimp. The crimped filament is then transferred to a special viewing holder by taping or gluing the ends so that about 10% slack is present and the filament length between the clamped ends is approximately 2.5 inches. The filament and viewing holder are then mounted vertically in a stoppered test tube containing desiccant. The tube is stored vertically overnight (18-24 hours) at 70° C. Following this conditioning period to dry the filament the tube is then brought to room temperature (approximately 25° C.). After allowing 30 minutes for cooling, the total number of crimps in the filament between the fixed ends is counted. In counting, any crimp reversal points present are ignored. The desiccant is then removed from the glass tube, the tube filled with water and stored vertically at 70° C. for 6 hours. The number of crimps in the wet fiber is counted as above. The cycles are repeated as required to obtain reproducible results. The equilibrium crimp reversibility (ECR) or relative change in crimps/inch of extended length from 25° C. dry to 70° C. wet is obtained by the following equation.

ECR =

$$\frac{\text{No. of crimps (25° dry)} - \text{No. of crimps (70° wet)}}{\text{No. of crimps (25° dry)}} \times 100$$

Alternatively the actual change in crimps/inch of extended length from 25° C. dry to 70° C. wet expressed as Δ c.p.i. may be used and is calculated as follows:

Δ c.p.i. =

$$\frac{(\text{ECR}) \text{ (crimps dry per inch of extended length dry)}}{100}$$

By extended length is meant the length of a filament or yarn as measured under sufficient tension to pull out the crimp and give an essentially straight filament or yarn. All crimp counts are stated in terms of extended length.

The crimp index of a fiber is determined on a sample that has been boiled in water and then dried in room temperature air. The length of the fiber under a load of 150 milligrams is determined ( $L_{150}$ ). This force is sufficient to straighten the fiber from crimps. The load on the fiber is then reduced to 5 milligrams and the crimped length ( $L_5$ ) determined. Crimp Index (C.I.) is calculated as follows:

$$\text{Crimp Index} = \frac{L_{150} - L_5}{L_{150}} \times 100$$

The crimp frequency is similarly determined on fibers that have been boiled in water and dried in room temperature air. The product of crimp index and crimp frequency is known as crimp product.

The necessary differential reversible length change between the components is readily obtained by altering the content of ionizable groups in the two polymers.

Such ionizable groups are readily obtained by copolymerizing acrylonitrile, for example, with monomers containing acid groups such as carboxylic, sulfonic or phosphonic in either the salt or free-acid form.

The following sulfonated polymerizable monomers and their salts are eminently suited for use in this invention: p-styrenesulfonic acid, methallylsulfonic acid, allylsulfonic acid and ethylenesulfonic acid.

It will be obvious to those skilled in the art that the required ionizable groups can be incorporated into a polymeric component by the blending of 2 or more polymers. The polymers should preferably be compatible.

The inclusion of from 1/2-15% of certain non-ionic modifiers in copolymers of acrylonitrile enhances the effect of any ionizable groups present in the final polymer. In general, it has been found that the monomers that are effective in this connection are also the same monomers which, when incorporated into an acrylonitrile polymer increases the dyeability of fibers made therefrom with a disperse dye, such as the blue-disperse dye Prototype 62.

Among the more desirable monomers from the point of view of enhancing the effect of ionizable group content are methyl acrylate, methyl methacrylate, methyl vinyl ketone, acrylamide, N-tertiarybutylacrylamide, vinyl methoxyethyl ether, methoxyethyl acrylate and vinyl acetate.

Pilling is a well-known phenomenon of fabrics made from staple fiber-yarns, and can be described as the tendency to form small clusters, clumps, or balls or intertangled fiber ends on the surface of a fabric. Pilling propensity can be measured by actual wear tests or by laboratory tests. The test described in the article, "Random Tumble Pilling Tester," by E. M. Baird et al. in Textile Research Journal 26, 731-735 (1956) is used herein.

The pilling ratings are expressed as numbers from -3 (very severe pilling) to +5 (no pilling). All times are for 20 minutes exposure unless otherwise stated.

Loop work-to-break. This is the area under the stress-strain curve of a loop of filament as determined on an Instron tester. The units are in gram-cm./denier-cm. This property and the elongation of a loop at break (loop elongation) are considered to be indicative of the toughness of the fiber.

The expression "intrinsic viscosity" with the symbol ( $n$ ) as used herein signifies the value of  $\ln(n)_r$  at the ordinate axis intercept (i.e., when  $c$  equals 0) in a graph of

$$\frac{\ln(n)_r}{c}$$

as ordinate with  $c$  values (grams per 100 ml. of solution) as abscissas. ( $n$ )<sub>r</sub> is a symbol for relative viscosity, which is the ratio of the flow times in a viscosimeter of a polymer solution and the solvent.  $\ln$  is the logarithm to the base  $e$ . All measurements on polymers containing acrylonitrile combined in the polymer molecule were made with DMF solutions at 25° C.

Referring to the drawings:

FIGURE 1 is a central cross-sectional elevation of a spinneret assembly which can be used to make the composite filaments of this invention;

FIGURE 1A is an enlarged portion taken from FIGURE 1 to show details of the spinneret at the spinning orifice;

FIGURE 2 is a transverse cross-sectional plan view of the apparatus of FIGURE 1 taken at 2-2 thereof and showing details of the top of the back plate;

FIGURE 3 is a transverse cross-sectional plan view

taken at 3-3 of FIGURE 1 showing details of the bottom of the back plate;

FIGURES 4, 5, and 6 show greatly magnified cross sections, i.e., sections perpendicular to the filament axis, of typical filaments of this invention produced by dry spinning. In these drawings one component is shaded to show the separation between components; and

FIGURE 7 is a schematic representation of apparatus that can be used in practicing the present process.

With reference to FIGURE 1, the bottom spinneret plate 2 which contains a circle of orifices 3 is held in place against back plate 1 by retaining rings 12 and 14 and by bolt 13. A fine-mesh screen 4 e.g., 200 mesh per inch, is pressed into position between, and serves as a spacer between, spinneret plate 2 and back plate 1. Back plate 1 contains two annular chambers 8 and 9 which are connected to suitable piping and filtration apparatus (not shown) to receive different spinning compositions. Lead holes 11 go from annular chamber 9 to annular space 7. Lead holes 10 lead from annular chamber 8 to annular space 6. Annular spaces 6 and 7 are separated by wall 5 which is disposed above orifices 3 and spaced from spinneret plate 2 by screen 4 to permit free and contiguous passage of the spinning fluids from annular spaces 6 and 7 through orifices 3, the mesh of screen 4 being fine enough to permit spinning fluid passage through orifices 3, as shown in detail in FIGURE 1A.

In FIGURE 2 are shown four lead holes 10 and four lead holes 11 equally spaced within the concentric chambers 8 and 9, respectively.

In FIGURE 3 are shown the concentric inner and outer annular spaces 6 and 7, sections of bottom spinneret plate 2 and the fine-mesh screen 4 partially in section.

Operation of the described apparatus in the practice of this invention is readily understood. Separate spinning materials are supplied to the inner annular chamber 9 and outer annular chamber 8, respectively, of the back plate; the former flows from chamber 9 through the lead holes 11 into the inner annular space 7 and thence through screen 4 and orifice 3 to form a part of a composite filament, while the latter passes through the lead holes 10 to the outer annular space 6 and thence through screen 4 and the outer side of the orifice 3 to form the other part of the composite filament.

FIGURE 7 is a schematic view of a wash-draw machine followed by a diagrammatic representation of a fluid relaxation chamber and a crimper. Tow 20 is drawn over rollers 25, 26 and through a series of water baths, 21, 22, 23, 24 while maintained under tension. This wash-draw treatment serves to extract solvent while the yarn is being drawn. The drawn yarn is then forwarded to a steam chest 28 for controlled relaxation and may then be passed directly to a crimper 30.

#### Example I

A 20% solution in dimethylformamide (DMF) of polyacrylonitrile of (n) 2.0 and containing 27 milliequivalents of acid groups per kilogram of polymer (as determined by titration in a DMF solution) is extruded into a spinning cell as one component (which faces the center of the spinning cell) of a composite filament using a spinneret as shown in FIGURE 1. Simultaneously, a 27% solution in DMF of a copolymer of acrylonitrile/styrenesulfonic acid, 96/4% by weight composition, of (n) 1.5 and analyzing 240 milliequivalents of acid per kilogram of polymer is extruded as the other component (which faces the wall of the cell) of composite filaments. The spinneret contains 140 orifices 0.007 inch in diameter located on a 5.27 inch diameter circle. A mixture of carbon dioxide and nitrogen gases at 320° C. is circulated through the spinning cell, the wall of which is maintained at 180° C. The solutions are extruded at 105° C. The threadline (1090 total denier) consisting of 140 composite filaments is wound up at 200 yards per minute (y.p.m.).

Three-hundred-thirty ends of yarn produced as above with a combined denier of 360,000 are combined into a tow and drawn to 4 times its original length (i.e., 4 × draw ratio) through a series of water baths at 95-98° C. which extract the residual DMF. The drawn and extracted tow is led directly from the wash-draw process to a stuffer box crimper similar to that shown in Hitt U.S. 2,747,233 where it is crimped to an extent of 6-7 herring bone crimps per extended inch using a stuffer box temperature of 50° C. The crimped tow is then cut into 3 1/8" length staple. The cut staple, loosely arranged in a tray, is dried for 15 minutes in a circulating air oven at 270-275° F. The dried staple (designated as Item A) has a weak mechanical crimp of 6-7 crimps per inch plus 6-8 helical crimps per inch of extended length.

The above process is repeated using the same components, spinning conditions and wash-draw conditions but with the significant change of placing an 8 foot long steam cell between the end of the wash-draw apparatus and the stuffer box crimper. The drawn and washed tow is passed into the steam cell containing steam at atmospheric pressure at a speed of 160 y.p.m. and is forwarded from the other end of the steam cell at 128 y.p.m. where it is fed continuously to the stuffer box crimper. The tow is relaxed to an extent of 20% in the steam cell during the 1.0 second time of exposure to the steam. The crimped tow is then cut and dried as above, to yield a product of this invention designated as Item B. The as-drawn yarn has a boil-off shrinkage of 21%.

Both Items A and B are fibers of good quality and have the following common properties after boiling in water: a density (as determined in a heptane-carbon tetrachloride gradient tube) of 1.189, an ECR value of about 40%, a tenacity of 2.2 grams per denier, a straight elongation at the break of 30%, and an initial modulus of 50 grams per denier. Other properties in which the two items vary significantly are shown in Table I.

Knitted fabrics are made from various spun yarns of the two items and the pilling resistance tested. The superior pilling properties of fabrics made from yarns of this invention (Item B) are surprising.

A third staple fiber is made as Item B using the steam cell but omitting the stuffer box crimper. Samples taken from the tow before the cutter are straight and uncrimped. These fibers that have not been mechanically crimped have essentially the same properties as Item B above.

Sweaters and woven fabrics made from the yarns of this invention (Item B) have a soft cashmere-like handle particularly when treated with a fiber lubricant. Fabrics of similar construction made from Item A have harsh handles similar to that of number 70's wool.

TABLE I

|                                                     | Item A | Item B |
|-----------------------------------------------------|--------|--------|
| Steam relaxed                                       | No     | Yes    |
| Helical crimps/inch                                 | 13     | 7      |
| Crimp index                                         | 10     | 5      |
| Residual shrinkage, percent                         | 3      | 1      |
| Loop elongation, percent                            | 10     | 17     |
| Loop, work to break                                 | 0.14   | 0.21   |
| Pilling ratings on knitted fabrics from:            |        |        |
| Worsted ply yarn (20/2 cotton count 14 Z/7 S twist) | -2.2   | +3.5   |
| Cotton singles (10 cotton count 8.5 Z)              | -3.0   | +2.5   |
| Woolen singles (5.1 wool run, 14 Z)                 | -2.5   | +0.5   |

The rating of -3.0 indicates very severe pilling as compared with +5 for no pilling.

Results similar to those of Item B are obtained when the wet drawn tow is fed into cans and lagged for 24 hours before passing through the steam cell. When using this batch method it is important that the stored tow be fed to the steam cell in an open form equivalent to that obtained from the draw machine.

A portion of the crimped tow of Item B is cut to 3-inch lengths and another portion is cut with lengths continuously varying from  $\frac{3}{4}$  to  $3\frac{1}{2}$  inch on a modified Beria staple cutter and dried. Worsted ply yarns (2/30 worsted count with an 8 Z/3.5 S turns per inch yarn twist) are spun from both lots of cut staple and knit tubing of similar construction prepared on a 12 cut Jacquard knitting machine. The fabric from 3-inch (square cut) staple has a pilling rating of 2.3 as contrasted with 4.5 for the fabric from the variable length staple. The advantages of using the variable length staple are even more striking with full fashion knit fabrics.

(dry, mechanically crimped staple) with 1 p.s.i. steam for 5 minutes, which develops crimp.

Items H to J are prepared from the above as-spun yarn by continuously drawing, passing through an 8 foot cell containing atmospheric steam, cutting to staple length and drying at  $130^{\circ}\text{C}$ . The speed of the output rolls is varied to control the amount of relaxation in the steam cell.

Similar cotton singles type yarns are spun from all items, fabrics of similar construction knitted and submitted to the pilling test for 20 minutes. The pilling ratings are given in Table II. The crimp per inch and density of the dry samples after boiling in water are given in Table II.

TABLE II

| Item | Steaming Conditions  | Steaming Relaxation, percent | Residual Shrinkage After Steaming | Density | Pilling | Crimps/inch |
|------|----------------------|------------------------------|-----------------------------------|---------|---------|-------------|
| E    | On piddled tow       | 20                           | 0-1                               | 1.160   | +1      | 14          |
| F    | On wet staple        | 20                           | 0-1                               | 1.159   | +1      | 14          |
| G    | On dry staple        | 3                            | 0-1                               | 1.185   | -2.0    | 13          |
| H    | On wet tow-tensioned | 0                            | 21                                | 1.189   | -3.0    | 12          |
| I    | do                   | 18                           | 13                                | 1.189   | +3.5    | 7           |
| J    | do                   | 20                           | 13                                | 1.190   | +3.5    | 7           |

### Example II

Composite filaments having as one component an 88/12% mixture (analyzing 55 milliequivalents of acid per kilogram of polymer) of polyacrylonitrile of (n) 2.0 and the copolymer acrylonitrile/sodium styrene sulfonate of 96.4% composition of (n) 1.5 and as the second component the above copolymer alone are prepared as in Example I except for the use of a spinning speed of 400 y.p.m. (instead of 200 y.p.m.) and the adjustment of the solution pumps to produce the same denier filaments as in Example I. The 4  $\times$  drawn, cut and dried ( $300^{\circ}\text{F}$ ) staple is designated as Item C. The as-drawn yarn has a boil-off shrinkage of 21%.

Item D is made as above except for the inclusion of the steam cell of Example I to provide 19% relaxation of the 40,000 denier tow between the wash-draw machine and the stuffer box crimper.

Both items of this example have high crimp reversibility (ECR of 40%) and a density of 1.185 after boiling in water.

The staple of Item C develops over 18 helical crimp per inch of extended length when boiled free of restraint in water. It has a crimp index of 18. Item D develops only 6 helical crimps per inch after boiling in water. It has a crimp index of 7.

Worsted ply yarns (20/2 cotton count, 11 Z/3.5 S twist) are spun from both items and knit fabrics of similar construction made. The fabric from Item C has a harsh raspy handle as contrasted with the soft and cashmere-like handle of the fabric from Item D. The latter fabric has an improved pilling rating over the fabric of Item C of 2 rating units.

### Example III

Composite filaments are extruded under the conditions of Example I, and 36 ends of the yarn combined to give a 40,000 denier tow which is drawn 4  $\times$  in a series of water tanks at  $95\text{--}98^{\circ}\text{C}$ . The water wet, drawn tow is piddled from side to side onto a continuous belt and then submitted to steam at atmospheric pressure for 2 minutes, which causes the tensionless tow to shrink about 20% and spontaneously crimp. The crimped tow is cut to staple length and dried with  $130^{\circ}\text{C}$ . air for 10 minutes to provide Item E.

Item F is prepared by passing the above drawn but uncrimped tow to a staple cutter and then depositing the wet staple on a continuous belt which is submitted to steam at atmospheric pressure and dry air at  $130^{\circ}\text{C}$ . in sequence which causes the filaments to crimp.

Item G is prepared by treating Item A of Example I

Those fibers having densities less than about 1.170 are very undesirable. They have a tendency to absorb an unusual amount of finish which may lead to odor difficulties in a final yarn. They take up a great deal of dye from a dye bath but yet yield a relatively low color in the yarn. Furthermore, in fabrics they display an instability in density which causes the appearance of dye streaks and luster streaks depending upon the pressure placed on the fabric in ironing procedures. To the contrary the fibers having a density of 1.180 to 1.200 are density stable and are not affected by these deficiencies.

It is surprising that the steaming process of this invention per se does not completely reduce the yarn shrinkage in this process. As the figures indicate, there is appreciable residual shrinkage before drying in such filaments and it is the high temperature drying step that sets the yarn and reduces shrinkage.

### Example IV

The spinning conditions of Example I are repeated to produce composite filaments having cross sections similar to those shown in FIGURE 6. 20 ends of the as-spun yarn are plied to give an 8000 denier tow which is then drawn a total of 2  $\times$  using the apparatus of Example I. The as-drawn yarn has a boil-off shrinkage of about 45%. The tow is then cut and dried on trays in an oven at  $130^{\circ}\text{C}$ . to form Item M.

Item N is formed using the same conditions as for M but with the inclusion of the steam cell of Example I and with the adjustment of the output rolls so that the tow has 0% relaxation during the steam treatment.

Item O is made in the same way as N with the exception that the tow is allowed to relax a total of 37% during the steaming operation.

The above three processes are repeated with the substitution of a 20% solution of polyacrylonitrile of (n) 2.0 and a 21% solution of the copolymer of Example I of (n) 2.0 to yield composite filaments having a cross section similar to FIGURE 5. Items P, Q, and R are obtained with no steam cell, 0% relaxation in the steam cell and 37% relaxation in the steam cell respectively.

The above processes yielding Items P, Q, and R are repeated with the reversal of the two spinning solutions in the spinning head so that the outer portion of the composite filament containing the homopolymer faces the wall of the spinning cell. This produces filaments of cross section similar to FIGURE 4. Items S, T, and U are obtained with no steam cell, 0% relaxation in the steam cell and 37% relaxation in the steam cell respectively.

Pilling ratings are determined from knit fabrics of

woolen single type yarns (5.1 run/8.52 twist) spun from the samples.

All items have an ECR of about 25-30% and other filament properties as shown in Table III after boiling in water.

5

The spinneret orifices are 0.007 inch in diameter. A mixture of carbon dioxide and nitrogen gases at 345° C. is circulated through the spinning cell, the wall of which is maintained at 200° C. The solutions are extruded at 120° C. The thread line (2,260 total denier, Item A;

TABLE III

| Item        | Cross Section   | Steaming Conditions | Crimps/inch | Residual Shrinkage, percent | Density | Loop Elongation, percent | Work to Break | Pilling Rating |     |     |
|-------------|-----------------|---------------------|-------------|-----------------------------|---------|--------------------------|---------------|----------------|-----|-----|
|             |                 |                     |             |                             |         |                          |               | 20'            | 30' | 60' |
| M, P, and S | Fig. 4, 5, or 6 | None                | 12          | 1.5                         | 1.189   | 9-13                     | 0.06          | -3             | -3  | -3  |
| N, Q, and T | Fig. 4, 5, or 6 | Taut 0% relax       | 20          | 3                           | 1.189   | 21                       | .36           | -3             | -3  | -3  |
| R           | Fig. 5-dogbone  | Tensioned 37% relax | 20          | 0                           | 1.189   | 64                       | .82           | -1             | +3  | +5  |
| U           | Fig. 4-dogbone  | do                  | 18          | 0                           | 1.187   | 48                       | -----         | -1             | 0   | +3  |
| O           | Fig. 6 acorn    | do                  | 18          | 0                           | 1.190   | 25                       | -----         | +3             | +5  | +5  |

## Example V

This example shows the advantages of the process of this invention with 1.35 X drawn fibers.

Fibers of the same composition as those in Example I are spun in the same manner except for spinning speeds of 400 y.p.m. and for the solution, head and cell temperatures of 60, 270 and 160° C. respectively. Four hundred fifty ends of the as-spun yarn (280 denier) are plied to give a 126,000 denier tow which is then drawn a total of 1.35 X using the apparatus of Example 1. The tow is then cut and dried on trays in an oven at 130° C. to form Item V.

Item W is formed using the same conditions as for V but with the inclusion of the steam cell of Example I and allowing the tow to relax a total of 20% during the steaming operation. The as-drawn fiber has a shrinkage of about 22%.

Both fibers developed a helical crimp of about 9 crimps per inch when boiled free from restraint in water and have a negative crimp reversibility of -30% ECR. Properties of the boiled-off fibers and knit fabrics prepared from them are given in Table IV.

TABLE IV

|                                                                                       | Item V | Item W |
|---------------------------------------------------------------------------------------|--------|--------|
| Density                                                                               | 1.184  | 1.189  |
| Loop Elongation, percent                                                              | 6.2    | 9.8    |
| Loop, Work to Break                                                                   | 0.06   | 0.09   |
| Pilling Ratings on Fabrics from: woolen-type yarn<br>5.1 run, 8.5 Z twist, 20 minutes | -1     | +5     |

Yarns made from Item W are significantly tougher than V as indicated by the loop properties. This results in improved knittability of these low tenacity fibers compared to Item V.

## Example VI

A 21% solution in dimethylformamide (DMF) of a mixture of 86% of polyacrylonitrile of intrinsic viscosity 2.0, and containing 22 milliequivalents of acid groups per kilogram of polymer (as determined by titration in a DMF solution) and 14% of a copolymer of acrylonitrile/styrene sulfonic acid, 96/4% by weight composition, of intrinsic viscosity 1.5, and analyzing 240 milliequivalents of acid per kilogram of polymer, said mixture of polymers containing 53 milliequivalents of acid groups per kilogram of polymer used, is extruded as one component (which faces the center of the spinning cell) of a composite filament using a spinneret having three concentric rings of orifices, totaling 252 in number. This solution also contains 0.04% TiO<sub>2</sub> based on total polymer content. Simultaneously, a 27% solution in DMF of a copolymer of acrylonitrile/styrene sulfonic acid, 96/4% by weight composition, of intrinsic viscosity 1.5, and analyzing 240 milliequivalents of acid per kilogram of polymer and also containing 0.4% TiO<sub>2</sub> based on total polymer content used, is extruded as the other component (which faces the wall of the cell) of composite filaments.

20,500 total denier, Item B) consisting of 252 composite filaments is wound up at 350 yards per minute.

Five-hundred seventy-six ends (Item A) or 635 ends (Item B) of yarn produced as above with a combined denier of 1,300,000 are combined into a tow and drawn to four times its original length (i.e., 4 X draw ratio) 25 through a series of water baths at 95-98° C. which extract the residual DMF, said water baths containing mixtures of DMF and water with not over 30% DMF.

For Item A, the drawn and extracted tow is led directly from the wash-draw process to a stuffer box crimper 30 similar to that shown in Hitt, U.S. 2,747,233, where it is crimped to an extent of six to seven herringbone crimps per extended inch using a stuffer box heated by steam at a pressure of 3 p.s.i.g. The crimped tow is then cut into staple of lengths continuously varying from 1 to 5 inches 35 on a modified Beria staple cutter. The cut staple is dried on a moving belt dryer at 140° C. for twenty-five minutes. The dried staple (designated as Item A) has a weak mechanical crimp of 5 to 6 crimps per inch plus 5 to 6 helix crimps per inch of extended length.

40 For Item B, the above process is repeated using the same components, spinning conditions, and wash-draw conditions, but with the significant change of placing an eight-foot long steam cell between the end of the wash-draw apparatus and the stuffer box crimper. The drawn and washed tow is passed into the steam cell, containing steam at atmospheric pressure, at a speed of 200 yards per minute where it is fed continuously to the unheated stuffer box crimper. The tow is relaxed to an extent of 15% in the steam cell during the 0.94 second time of exposure to the steam. The crimped tow is then cut and dried as above, to yield a product of this invention designated as Item B.

Items A and B have the following common properties after boiling in water: a density (as determined in heptane-carbon tetrachloride gradient tube) of 1.189, an ECR value of 30%, a tenacity of 2.5 g.p.d., and a straight elongation at break of 32%. Properties in which the two items vary significantly are shown in Table V.

TABLE V

|                                                                                        | Item A | Item B |
|----------------------------------------------------------------------------------------|--------|--------|
| Steam relaxed                                                                          | No     | Yes    |
| Helical Crimps/in. (Boiled, air-dried, 25° C.)                                         | 12     | 8.5    |
| Crimp Index (Boiled, air-dried, 25° C.)                                                | 11     | 7      |
| Residual Shrinkage, percent                                                            | 4.2    | 2.4    |
| Initial Modulus, g.p.d.                                                                | 42     | 53     |
| Loop Elongation, percent                                                               | 9.0    | 10.5   |
| Loop Work-to-break                                                                     | 0.11   | 0.14   |
| Pilling Rating in Knitted Fabrics from: Worsted<br>Ply Yarn (20/2 cc., 14 Z/7 S twist) | 1.0    | 3.5    |

70 What is claimed is:

1. In a process for preparing staple fiber from composite filaments, the resulting staple fiber having improved resistance to pilling which comprises simultaneously washing and drawing a tow of continuous filaments wherein 75 said filaments have two eccentrically positioned sections

of different acrylonitrile polymers extending along their lengths, the improvement which comprises a controlled relaxation step provided by continuously passing said filaments under a slight tension through a heated plasticizing medium, the tension on said filaments and the temperature of said medium being controlled to uniformly shrink said filaments an amount equal to at least 50% of the boil-off shrinkage of said drawn filaments, and converting the resulting tow of relaxed continuous filaments to staple fiber and drying the staple fiber at high temperature.

2. The process of claim 1 wherein said tension is at least 0.01 gram per denier and said composite filaments each have a section of polyacrylonitrile eccentrically positioned with respect to a section of an acrylonitrile/styrene-sulfonic acid copolymer.

3. The process of claim 1 wherein said filaments are drawn from about 1.1 to 10 times their original length and after shrinking are crimped.

4. The process of claim 1 wherein said medium is steam.

5. The process of claim 1 wherein the relaxation treatment under tension is carried out in the presence of steam at about 0 to 5 p.s.i. gage.

## References Cited by the Examiner

## UNITED STATES PATENTS

|    |           |         |                 |           |
|----|-----------|---------|-----------------|-----------|
| 5  | 2,428,046 | 9/1947  | Sisson et al.   | 28—82     |
|    | 2,439,814 | 4/1948  | Sisson          | 28—82     |
|    | 2,810,281 | 10/1957 | Appleton et al. | 28—72 X   |
|    | 2,917,805 | 12/1959 | Rokosz          | 28—72     |
|    | 2,917,806 | 12/1959 | Spence et al.   | 28—72     |
| 10 | 3,003,222 | 10/1961 | Pitzl           | 28—72     |
|    | 3,017,686 | 1/1962  | Breen et al.    | 161—177 X |
|    | 3,038,237 | 6/1962  | Taylor          | 161—172   |
|    | 3,038,238 | 6/1962  | Wu              | 161—175   |

## FOREIGN PATENTS

|    |         |         |                |
|----|---------|---------|----------------|
| 15 | 760,179 | 10/1956 | Great Britain. |
|----|---------|---------|----------------|

ROBERT R. MACKEY, Primary Examiner.

RUSSELL C. MADER, DONALD W. PARKER,  
Examiners.J. B. MAIER, A. J. SMEDEROVAC,  
Assistant Examiners.